

## UNITED STATES PATENT OFFICE

WALTER SEIDEL AND ALBERT ERNECKE, OF DORMAGEN, GERMANY, ASSIGNEES TO  
I. G. FARBNINDUSTRIE AKTIENGESELLSCHAFT, OF FRANKFORT-ON-THE-MAIN,  
GERMANY, A CORPORATION OF GERMANY

## ARTIFICIAL THREAD

No Drawing. Application filed April 5, 1929, Serial No. 352,906, and in Germany April 12, 1928.

- The present invention relates to a process of improving artificial silk prepared from cellulose acetate and to the products obtained thereby.
- According to our invention the tensile strength of artificial silk prepared from cellulose acetate according to the dry spinning process can be highly increased by impregnating the threads with a diluted organic fatty acid having not more than three carbon atoms, that means by impregnating the cellulose acetate with a diluted acid of the group consisting of formic-, acetic- and propionic acids and stretching the threads from about 50% to about 400% of their length. The concentration and the temperature of the diluted acids used in our process may be varied, but care must be taken that the threads are not caused to stick together; the concentration somewhat depends on the temperature at which the process is carried out, generally we work with an acid having a concentration between about 30% and about 45% and a temperature from about 15° to about 30° C.; the lower the temperature the higher must be the concentration of the acid. The threads after having been stretched according to our process are washed with water until free from acid and dried; advantageously the threads are kept in tension during the washing and drying process by attaching a weight thereto. As in stretching the threads the liquid is pressed out, care must be taken that during the whole stretching process diluted acid is present, for example by irrigation with said diluted acids. The best results are obtained in our process if the removing of the acid is performed in stages, that will say, the stretching is not completely performed with an acid of about 30 to about 45%, but, after a partial stretching the concentration of the acid, the threads are irrigated with, is diminished to about 25%, after a further stretching the concentration is diminished to about 20%; the stretching is completed with an acid of about 10% strength.
- Our process may be carried out either directly after the spinning process by treating the single threads according to our new process; but generally we use for the purpose of our invention cellulose acetate silk in form of ropes, the threads of which may be twisted or untwisted.
- Artificial threads prepared from cellulose acetate according to the dry spinning process have an average tensile strength of 100 to 120 grams per 100 deniers, sometimes up to 150 grams. By treating cellulose acetate threads according to our new process their tensile strength is highly increased and the diameter of the thread is diminished.
- The invention is illustrated by the following examples, without being limited thereto:
- Example 1.*—A rope of cellulose acetate silk prepared according to the dry spinning process having in the dry state a tensile strength of 100 grams per 100 deniers and in the moist state a tensile strength of 50 grams per 100 deniers and the threads having a titer of 7 deniers, is impregnated with a 40% acetic acid of about 18° C. and extended by slowly stretching to three times its length. During the stretching the rope is irrigated with 40% acetic acid the concentration of which is by and by decreased; when the stretching is complete, the rope is washed with water and dried, a tension thereby being maintained by appending a weight to the rope. The threads thus obtained have in the dry state a tensile strength of more than 240 grams per 100 deniers, in the moist state a tensile strength of more than 150 grams per 100 deniers, the titer of the thread is 2.2 deniers.
- Example 2.*—A rope of cellulose acetate silk is impregnated with a 35% aqueous formic acid of 20° C., and is then stretched to about 200%; then the acid is removed in stages while maintaining the tension of the threads; the acetate silk is washed and dried as described in Example 1. It has the same properties as that of Example 1.
- We claim:
1. The process which comprises impregnating artificial silk which has been prepared from cellulose acetate according to the dry spinning process with an aqueous solution of a fatty acid of the group consisting of formic, acetic, and propionic acids of 30 to 45%.

95  
100

strength and having a temperature from 15 to 30° C. and stretching the artificial silk from 50 to 400% its length, washing and drying the same.

5 2. The process which comprises impregnating artificial silk which has been prepared from cellulose acetate according to the dry spinning process with an aqueous solution of a fatty acid of the group consisting of 10 formic, acetic, and propionic acids of 30 to 45% strength and having a temperature from 15 to 30° C. and stretching the artificial silk from 50 to 400% its length, removing the acid in stages and drying the artificial silk.

15 3. The process which comprises impregnating artificial silk which has been prepared from cellulose acetate according to the dry spinning process with an aqueous acetic acid of about 40% strength and having a temperature from 15 to 30° C. and stretching the artificial silk from 50 to 400% its length, washing and drying the same.

20 4. The process which comprises impregnating artificial silk which has been prepared from cellulose acetate according to the dry spinning process with an aqueous acetic acid of 40% strength and having a temperature from 15 to 30° C. and stretching the artificial silk from 50 to 400% its length, removing the acid in stages and drying the artificial silk.

25 5. The process which comprises impregnating a rope of artificial silk which has been prepared from cellulose acetate according to the dry spinning process with an aqueous solution of a fatty acid of the group consisting of formic, acetic, and propionic acids of 30 to 45% strength and having a temperature from 15 to 30° C. and stretching the rope from 50 to 400% its length, washing and drying the same.

30 6. The process which comprises impregnating a rope of artificial silk which has been prepared from cellulose acetate according to the dry spinning process with an aqueous solution of a fatty acid of the group consisting of formic, acetic, and propionic acids of 30 to 45% strength and having a temperature from 15 to 30° C. and stretching the rope from 50 to 400% its length, removing the acid in stages and drying the rope.

35 7. The process which comprises impregnating a rope of artificial silk which has been prepared from cellulose acetate according to the dry spinning process with an aqueous acetic acid of 40% strength and having a temperature of about 18° C. and stretching the rope from 50 to 400% its length, washing and drying the same.

40 8. The process which comprises impregnating a rope of artificial silk which has been prepared from cellulose acetate according to the dry spinning process with an aqueous acetic acid of 40% strength and having a temperature of about 18° C. and stretching

the rope from 50 to 400% its length, removing the acid in stages and drying the artificial silk.

In testimony whereof we have hereunto set our hands.

WALTER SEIDEL. [L. S.]  
ALBERT ERNECKE. [L. S.]

70

75

80

85

90

95

100

105

110

115

120

125

130